

# UNITED STATES PATENT OFFICE.

WILTON E. DARROW, OF SUTTER CREEK, CALIFORNIA.

## PROCESS FOR TREATING CYANIDABLE ORES CONTAINING DELETERIOUS SLIMES.

1,098,020.

Specification of Letters Patent.

Patented May 26, 1914.

No Drawing.

Application filed March 11, 1914. Serial No. 823,976.

*To all whom it may concern:*

Be it known that I, WILTON E. DARROW, a citizen of the United States, residing at Sutter Creek, in the county of Amador, State of California, have invented certain new and useful Improvements in Processes for Treating Cyanidable Ores Containing Deleterious Slimes; and I do declare the following to be a full, clear, and exact description of the 10 same.

This invention relates to an improved process for the treatment of crushed ores. In the cyanidation of gold ores, it is sometimes found that the slimed portions of the 15 crushed ore contain graphite or other deleterious substances which act as precipitants thus causing an actual loss of values in the treatment of the ores or which slimed portions containing such deleterious substances 20 are of such low value as to be commercially valueless for treatment. I have discovered from years of experiment that many of these ores can be profitably cyanided by first separating the granular particles from the 25 slimed portion; which slimed portion contains the greater portion of the deleterious compounds and then by subjecting such slimed portion to a concentration process the greater portion of its contained gold can be 30 obtained in enriched cyanidable concentrates which are nearly free from the graphite and deleterious colloidal substances. This elimination of the colloidal slime and graphite 35 removes also the greater portion of acidity from the ore thus effecting a great saving of

the quantity of chemicals used in the subsequent cyanidation of the enriched product.

The various steps in my improved process for the treatment of the ores consist in passing the crushed ore through a succession of cone classifiers with intermediate dilutions of clear water or other similar classification means might be used. By this means the slimed portions are removed in that form from the granular particles. Such slimed 40 portions are then concentrated preferably by means of being washed over concentrating tables of suitable construction whereby the deleterious graphite or other colloidal substances are removed, the greater portion of 45 the associated gold being collected on the tables in fairly clean and cyanidable concentrates. These concentrates and the granular portions are then subjected to cyanidation in any suitable manner. 50

Having described the steps of my improved process what I claim is:

The herein described process of treating cyanidable crushed ores consisting in first separating the granular particles and the 60 slimes of said ores and then treating the slimed portion thereof to remove therefrom the graphite and other deleterious colloidal substances, as described. 65

In testimony whereof I affix my signature in presence of two witnesses.

WILTON E. DARROW.

Witnesses:

STEPHEN H. BLEWETT,  
FLOYD M. BLANCHARD.

Copies of this patent may be obtained for five cents each, by addressing the "Commissioner of Patents, Washington, D. C."